

Dec. 8, 1925.

1,564,732

J. WEATHERBY

METHOD AND APPARATUS FOR SEPARATING ORE PARTICLES

Original Filed July 21, 1922



Fig. 1.

Fig. 2.



Fig. 3.

Fig. 4.



Inventor:

Joseph Weatherby,  
By Church & Church

His Attorneys:

## UNITED STATES PATENT OFFICE.

JOSEPH WEATHERBY, OF HARRISBURG, PENNSYLVANIA, ASSIGNOR TO WEATHERBY ORE SEPARATOR COMPANY, OF PHILADELPHIA, PENNSYLVANIA, A CORPORATION OF DELAWARE.

## METHOD AND APPARATUS FOR SEPARATING ORE PARTICLES.

Original application filed July 21, 1922, Serial No. 576,622. Divided and this application filed February 4, 1924. Serial No. 690,582.

To all whom it may concern:

Be it known that I, JOSEPH WEATHERBY, a citizen of the United States, residing at Harrisburg, in the county of Dauphin and State of Pennsylvania, have invented certain new and useful Improvements in Method and Apparatus for Separating Ore Particles; and I do hereby declare the following to be a full, clear, and exact description of the same, reference being had to the accompanying drawings, forming part of this specification.

My invention relates to an improved method of separating ore particles from their gangue, and one ore from another, depending on their susceptibility to alternating current magnetic flux and their permeable or non-permeable qualities, this application being a division of my pending application Serial No. 576,622, filed July 21, 1922, entitled "Method of separating ore particles."

My invention more particularly relates to the separation of ore particles from their gangue and of one particular ore from another, by the use of multi-phase alternating current in the type of magnetic separator shown in drawings attached and described in the following specification.

In the drawings—

Figure 1 is a perspective view of the multi-phase alternating current field magnet under the ore feed board.

Figure 2 shows two multi-phase alternating current magnets mounted above an ore feed board with an armature for the lower field magnet mounted below it and under the ore feed board.

Fig. 3 shows the diamond shaped overlapping coils of the field magnets where one side of the coil is in the top of one slot of the field magnet, and the other side of the coil in the bottom of a further slot to form north and south poles, and also showing the electrical connections suitable for three phase alternating current.

Fig. 4 shows a section of an armature with its single pole wound coils and electrical connections.

Figure 1 shows an ore feed board 45

adjustably mounted on adjusting bolts 37 above a field magnet composed of a plurality of units 26. The device is on such a slant that if granular ore is fed to the top 64 of the feed board it will flow by gravity to and over the bottom edge 65 of the board to a discharge (not shown). Now if a multi-phase alternating current is switched on the magnet 25 through coils connected so that the rotating or progressing field will travel from right to left and if an ore feed is arranged at the upper right hand corner of this magnet and dropped on the ore feed board 45 the gangue or non-metallic particles will flow down the right hand side 65 and over the edge 65 of the bottom of the board, while the metallic particles will take an electrical charge due to the alternating magnetic flux passing from the field magnet up through them. These particles, if permeable magnetically, will be attracted toward the board 45 and be forced to move with the rotating magnetic field to the left of the board and away from the gangue material and will be discharged at the bottom by 70 weakening the current in the last few coils in a tapering way to a point where the ore is not susceptible so that these magnetically permeable particles will flow off the board at the lower left hand corner while those 80 particles which are metallic and not permeable magnetically will be repelled in the reverse direction to and over the right edge of the feed board.

It might here be noted that every ore particle no matter how fine it is ground to a powder, takes its own individual electrical charge in the field and acts entirely as its own agent independent of its neighbor in the rapid travel following the rotating alternating current field, and therefore spins and gyrates in its travel throwing all other particles away from it.

In Fig. 2 are shown two field magnets with their adjustable spacer boards 40 95 mounted above a feed board 45. The top magnet does not have an armature, but the lower field magnet has an armature 30 swung below the feed board. The upper field is arranged to discharge its concen- 100

- trate on one side while the lower field magnet discharges its concentrate on the other side of the feed board 45. This arrangement is used to remove a magnetic susceptible substance from a non-magnetic metallic substance, and both from a gangue material. Or by this arrangement one magnetic ore can be separated from another magnetic ore of a lesser susceptibility. If an ore particle's responsive frequency is faster than that of another ore particle it can be separated from such other ore particles by the fact of it responding to magnetic attraction away from the reluctant particle. The ore particle will be quick or sluggish dependent upon the frequency that energizes it and if its responsive frequency is lower than the frequency that energizes it, then it will lag to the alternating magnetic attractions.
- As above stated, the field magnet 25 can be used without an armature 30, the object of the armature being merely to intensify or concentrate the magnetic field to improve the power factor and further to increase the distance in which ore is susceptible to the field influence.
- The field magnet has coils and is connected as shown in section Fig. 3, while the armature 30 has single pole coils and is connected as shown in Fig. 4. It will be noted that the diamond shaped coils on the field magnet are connected three phase star multiple. It is just as well to state here that the coils may be connected in any of the well known ways, such as in star series, delta, delta series, etc. It will also be noted that the armature coils in Fig. 4 are in part connected series star while the rest are closed circuited. Either type can be used on either armature or field to meet different conditions in the ore to be separated, as each type has peculiar features that can be used advantageously in various ways.
- In the following description I describe the diamond overlapping coil on the field and the single pole coil on the armature, this being the preferable construction. Now consider that a three phase alternating current has been switched on the field magnet and current is flowing in all the coils A, B and C, etc. An adjustable resistance or an impedance is used on the last few coils of the field magnet to taper their magnetic strength in such a way that each following tooth or pole is weaker in magnetic strength than the one before it. This is done to permit magnetic susceptible ore particles to be released and to drop away from the rotating or progressing field. This is not necessary in the case of non-magnetic metallic substances as they are repelled by and away from the rotating field, while the magnetic substances are attracted to and advance with the rotating field.

No provisions have as yet been made for the connection of the terminal wires leading from the armature with the exception that the coils on the last three teeth or poles of the armature have their terminals short circuited or closed. Current is now flowing in all the field coils and all the teeth or poles are energized with a rotating magnetic field.

Magnetic flux is now flowing through the field magnet out the tips of the poles or teeth and across the air gap to the armature teeth through the armature, back through the teeth and air gap to the field poles or teeth again. This sets up a strong magnetic field in the armature teeth by induction which rotates in step with that of the field magnetism that energizes it. The current is alternating, therefore the magnetic flux alternates back and forth across the air gap at a speed equal to the frequency and the poles or teeth of both the field magnet and the armature reverse their polarity changing from north to south and back to north again very rapidly, as for instance in 60 cycle current they would change polarity 7200 times per minute.

When the coils on the armature are open circuited no current flows through them. The armature iron is magnetized by the field flux flowing through it. Magnetic permeable particles have a tendency to bridge between the armature poles and the field poles, even though they are spinning in step with the frequency.

When the armature coils are in a closed circuit as shown in the last three coils of Fig. 4, current flows in them causing a counter flux to be set up in the armature which opposes the field flux that energizes it, thus causing the permeable ore particles to be repelled in the direction of the field poles as they travel with the rotating field.

Since non-magnetic metallic substances are repelled away from the magnetic field in any case, it makes little difference whether the armature coils are open or closed for non-magnetic metallic substances. By intermittently opening and closing the armature coils permeable ore particles are caused to jump up and down violently during their progression, as well as to spin thus freeing themselves from the gangue material which tends to adhere to them.

It will now be considered that all the armature are in a closed circuit and that the field magnets are tilted to such an angle that ore will freely flow down the feeder board 45 in the air gap between the field and armature, to a discharge.

It is to be noted that there are no moving parts on this type of separator and that all ore moves by gravity alone, or is forced to travel with or against gravity by the rotating magnetic field.

The gate of the hopper (not shown) is now opened and a granular stream of ore permitted to flow to the feeder board 45. The gangue material which is non-metallic and is not affected by the alternating current flux, flows down the feeder board to its discharge at the bottom.

The permeable magnetic particles on entering the field even though they are as fine as dust, have natural polarity and will start to spin rapidly when the alternating flux passes through them trying to present their poles in proper relation to the lines of force, thus freeing themselves from gangue material, and one from the other. They are also repelled from the armature poles and in the direction of the field poles and they are influenced to travel with the rotating magnetic field. They travel down on the under side of spacer board 40 at great speed, much faster than the gangue that is flowing by gravity on the feeder board 45. When they reach the bottom of the spacer board 40 as the current in the lower coils is tapered and weakened, they drop away from the rotating field to the discharge.

It often happens that magnetic materials are sluggish and will not travel in step with the rotating field dropping back in phase or slipping, and in such a case it is required that a more violent agitation be imparted to the magnetic material traveling with the rotating field. In such a case it is arranged that the armature coils be intermittently opened and closed, which causes the ore particles to violently jump up and down between armature and field as well as spin while they are traveling to their discharge with the rotating field currents, as the armature is first attractive when the coils are opened and then repellent when the coils are closed.

What I claim is:

1. The art of electrically separating permeable particles from gangue which consists in passing a mixture of particles and gangue between a progressive multi-phase magnetic field and an induced field.

2. The art of electrically separating two permeable particles from each other and from gangue which consists in passing a mixture of particles and gangue past two progressive multi-phase fields of different strengths.

3. The art of separating magnetic particles from gangue which consists in passing the mixture of particles and gangue across a multi-phase progressive field which moves transversely to the path of the mixture, in increasing the frequency of said field until maximum movement of the particles is secured, and in continuing the current in the field at said responsive frequency.

4. The art of separating magnetic ore particles from gangue which consists in

passing a mixture of gangue and particles between a multi-pole electro-magnet and an armature, said magnet having a multi-phase progressive magnetic field transversely moving with respect to the path of said mixture, 70 said armature being particle attractive at its receiving end and being particle-repellent at its discharge end.

5. The art of electrically separating permeable particles from gangue which consists in passing the mixture of particles and gangue between two insulating surfaces and through a progressive field moving transversely to the path of the mixture.

6. The art of electrically separating permeable particles from gangue which consists in passing the mixture of particles and gangue through an edge only of the progressive field moving transversely to the path of the mixture.

7. The art of electrically separating permeable particles from gangue which consists in passing the mixture of particles and gangue through the curved portions only of the lines of force of a progressive field moving transversely to the path of the mixture.

8. The art of electrically separating permeable particles from gangue which consists in passing the mixture of particles and gangue between two progressive fields moving transversely to the path of the mixture while restraining said mixture from crossing the straight and nearly straight portions of the lines of force of each of said fields.

9. The art of electrically separating permeable particles from gangue which consists in passing the mixture of particles and gangue between two non-metallic surfaces and from a progressive field whereby the mixture is caused to move in the edge only of said field, and the magnetic particles are caused to travel along the upper of said surfaces and to move transversely to the path of the gangue.

10. The art of electrically separating two magnetic ores of different susceptibility from each other and from gangue, which consists in passing the mixture of particles and gangue down a gravity chute and successively under progressive fields of different strengths, one field moving to the right with respect to the chute and the other field moving to the left whereby the gangue will pass down the chute, the particles of one ore will pass to one side of the chute, and the particles of the other ore will pass to the other side of the chute.

11. The art of separating magnetic ore particles from gangue, which consists in passing a mixture of gangue and particles beneath a non-metallic board beneath a magnet having a progressive multi-phase field, whereby the magnetic particles will rise against gravity from the path of the

- gangue and will follow said field to one side of said travel of the gangue and out of contact therewith.
12. The art of separating magnetic ore particles from gangue, which consists in passing a mixture of gangue and particles between a multi-pole electromagnet and an armature, said magnet having a multi-phase progressive magnetic field moving transversely with respect to the path of the mixture, said armature being particle attractive beneath the path of the mixture, and being particle repellent in the path of the particles beyond the path of the gangue.
13. The process of claim 12 in which the magnet has its coils tapered, so that each successive path or pole is weaker in magnetic strength than the one before it.
14. In combination, a sloping feed board, a spacer board arranged transversely of, 20 and spaced above said feed board, a multi-phase alternating current above said spacer board and extending to one side thereof, the coils of said field magnet being tapered in magnetic strength so that each pole decreases in magnetic strength in accordance with its distance to one side of said feed board 25
15. In a device for separating permeable particles from gangue, a non-magnetic feed chute, a plurality of spacer boards, a multi-phase alternating current magnet above each spacer board, one of said magnets extending to the right of the feed chute, and the other extending to the left, and each magnet 30 35 adapted to produce a traveling field transversely of the feed chute.

JOSEPH WEATHERBY.